

2 Sheets—Sheet 1.

J. R. WILLIAMS.  
Manufacture of Horseshoes.

No. 225,259.

Patented Mar. 9, 1880.



Fig 2.



Attest:  
Geo. T. Smallwood Jr.  
Walter Allen

Inventor:  
John R. Williams  
By Knight Bros  
Otter.

2 Sheets—Sheet 2

J. R. WILLIAMS.

Manufacture of Horseshoes.

No. 225,259.

Patented Mar. 9, 1880.

Fig 3,



Fig 4,



Inventor:

John R. Williams  
By Knight Bros  
Atty:

Attest:

Geo. T. Smallwood Jr.  
Walter Allen

# UNITED STATES PATENT OFFICE.

JOHN R. WILLIAMS, OF JOHNSTOWN, PENNSYLVANIA, ASSIGNOR TO  
CAMBRIA IRON COMPANY.

## MANUFACTURE OF HORSESHOES.

SPECIFICATION forming part of Letters Patent No. 225,259, dated March 9, 1880.

Application filed August 18, 1879.

*To all whom it may concern:*

Be it known that I, JOHN R. WILLIAMS, of Johnstown, in the county of Cambria and State of Pennsylvania, have invented new and useful Improvements in the Manufacture of Horseshoes, of which the following is a specification.

The subject of this invention is a calked horseshoe produced in steel in one piece without welding, the calks being hardened, especially 10 at their points, to render them durable, and the body of the shoe being annealed to render it strong and not liable to break.

In the accompanying drawings, Figure 1 is a plan view of the under side of a calked horseshoe illustrating my invention. Fig. 2 is a vertical section of the same on the line 22, Fig. 1. Figs. 3 and 4 are sectional views, showing the shoe in the chemical and water baths, illustrating the mode of carrying my invention into effect, as hereinafter described.

B represents the body of the shoe; C C, calks, of pyramidal or other tapering shape, formed thereon; and D, the customary toe-clip.

The mode of rolling calked-horseshoe bars 25 from suitable bars or billets of steel is described and shown in my Letters Patent No. 182,732, dated September 26, 1876. The bar, having been thus suitably formed, is creased and trimmed and bent and finished, as I have 30 described in several applications now pending in the United States Patent Office. By thus producing the calked blank and the calked shoe I obtain calks formed in one piece from the solid bar and a horseshoe that is in one 35 solid piece without welding in any of its parts.

The calked shoe, having been thus made, is tempered unequally by the following process: The shoe is heated to a cherry-red, and, being taken from the fire by means of tongs, is set 40 in upright position—that is to say, with the calks downward—in a mixture, E, of equal parts of prussiate of potash, saltpeter, and sal-ammoniac in a finely-pulverized state, lying about one-quarter of an inch deep on a plate, F, as 45 illustrated in Fig. 3. The calks of the shoe are allowed to rest in this mixture for a few seconds,

and are then immersed in water, by means of the apparatus shown in Fig. 4, without immersing the body B of the shoe. To effect this object I employ a rack or frame, G G, consisting of bars at a sufficient distance apart to admit the calks between them, and extending across a suitable vessel, H, containing water, the water being allowed to fill the vessel up to the level of the top of the bars G, or nearly 50 so, so as to cool the calks C C, which project downward between the bars, without cooling, by actual contact, the body B of the shoe, the said body B being at this stage much too hot to be annealed by water. The bars permit the 55 calks of the shoe to project down between them into the water, as shown; but the water in the vessel should not cover the supporting-bars G; otherwise the body B of the shoe is liable to be too rapidly cooled, and consequently 60 hardened. The shoe is allowed to rest on these bars with the calks in the water until the body B is reduced to the annealing heat by spontaneous cooling, the required heat being a 65 dark-red color in the dark. When the body 70 has reached a sufficiently low temperature by spontaneous cooling it is plunged into water and cooled, which completes the operation and produces a calked horseshoe with hardened calks and an annealed body. 75

Having thus described my invention, the following is what I claim as new therein and desire to secure by Letters Patent:

1. A calked horseshoe composed of steel in one piece, with the calks C hardened and the 80 body B annealed, as hereinbefore described.

2. The processes of hardening the calks and annealing the body of a calked horseshoe by preliminary treatment with chemicals, sudden cooling of the calks only by immersing them 85 in water, and subsequent cooling of the whole after the body has reached the annealing temperature, substantially as herein set forth.

JOHN R. WILLIAMS.

Witnesses:

CYRUS ELDER,  
ROBERT P. FIELD.